# EUROPEAN PATENT SPECIFICATION

(11) **EP 3 027 363 B1**
(45) Date of publication and mention of the grant of the patent: **15.01.2020**
(21) Application number: 14747270.8
(22) Date of filing: 17.07.2014
(51) Int. Cl.: B24B 37/24

(54) **LOW DENSITY POLISHING PAD**
POLIERKISSEN MIT NIEDRIGER DICHTE
TAMPON DE POLISSAGE À FAIBLE DENSITÉ

(30) Priority: 31.07.2013 US 201313955398
(43) Date of publication of application: 08.06.2016
(73) Proprietor: Cabot Microelectronics Corporation, Aurora, Illinois 60504 (US)
(72) Inventor: HUANG, Ping, Beaverton, Oregon 97006 (US); ALLISON, William C., Beaverton, Oregon 97006 (US); FRENTZEL, Richard, Murrieta, California 92563 (US); LEFEVRE, Paul Andre, Portland, Oregon 97229 (US); KERPRICH, Robert, Portland, Oregon 97229 (US); SCOTT, Diane, Portland, Oregon 97212 (US)
(74) Representative: J A Kemp LLP
(86) International application number: PCT/US2014/047065
(87) International publication number: WO 2015/017138

(56) References cited:
- WO-A1-2013/058183
- US-A- 5 885 312
- US-A1- 2012 094 586

## Description

### TECHNICAL FIELD

Embodiments of the present invention are in the field of chemical mechanical polishing (CMP) and, in particular, low density polishing pads and methods of fabricating low density polishing pads.

### BACKGROUND

Chemical-mechanical planarization or chemical-mechanical polishing, commonly abbreviated CMP, is a technique used in semiconductor fabrication for planarizing a semiconductor wafer or other substrate.

The process involves use of an abrasive and corrosive chemical slurry (commonly a colloid) in conjunction with a polishing pad and retaining ring, typically of a greater diameter than the wafer. The polishing pad and wafer are pressed together by a dynamic polishing head and held in place by a plastic retaining ring. The dynamic polishing head is rotated during polishing. This approach aids in removal of material and tends to even out any irregular topography, making the wafer flat or planar. This may be necessary in order to set up the wafer for the formation of additional circuit elements. For example, this might be necessary in order to bring the entire surface within the depth of field of a photolithography system, or to selectively remove material based on its position. Typical depth-of-field requirements are down to Angstrom levels for the latest sub-50 nanometer technology nodes.

The process of material removal is not simply that of abrasive scraping, like sandpaper on wood. The chemicals in the slurry also react with and/or weaken the material to be removed. The abrasive accelerates this weakening process and the polishing pad helps to wipe the reacted materials from the surface. In addition to advances in slurry technology, the polishing pad plays a significant role in increasingly complex CMP operations.

However, additional improvements are needed in the evolution of CMP pad technology.

### SUMMARY

Embodiments of the present invention include methods of fabricating low density polishing pads.

### BRIEF DESCRIPTION OF THE DRAWINGS

Figure 1A is a top down view of a POLITEX polishing pad, in accordance with the prior art.
Figure 1B is a cross-sectional view of a POLITEX polishing pad, in accordance with the prior art.
Figures 2A-2G illustrate cross-sectional views of operations used in the fabrication of a polishing pad, in accordance with an embodiment of the present invention.
Figure 3 illustrates cross-sectional views at 100x and 300x magnification of a low density polishing pad including closed cell pores which are all based on a porogen filler, in accordance with an embodiment of the present invention.
Figure 4 illustrates cross-sectional views at 100x and 300x magnification of a low density polishing pad including closed cell pores, a portion of which based on a porogen filler and a portion of which is based on gas bubbles, in accordance with an embodiment of the present invention.
Figure 5A illustrates a plot of population as a function of pore diameter for a broad mono-modal distribution of pore diameters in a low density polishing pad, in accordance with an embodiment of the present invention.
Figure 5B illustrates a plot of population as a function of pore diameter for a narrow mono-modal distribution of pore diameters in a low density polishing pad, in accordance with an embodiment of the present invention.
Figure 6A illustrates a cross-sectional view of a low density polishing pad having an approximately 1:1 bimodal distribution of closed-cell pores, in accordance with an embodiment of the present invention.
Figure 6B illustrates a plot of population as a function of pore diameter for a narrow distribution of pore diameters in the polishing pad of Figure 6A, in accordance with an embodiment of the present invention.
Figure 6C illustrates a plot of population as a function of pore diameter for a broad distribution of pore diameters in the polishing pad of Figure 6A, in accordance with an embodiment of the present invention.
Figure 7 illustrates an isometric side-on view of a polishing apparatus compatible with a low density polishing pad, in accordance with an embodiment of the present invention.

### DETAILED DESCRIPTION

Low density polishing pads and methods of fabricating low density polishing pads are described herein. In the following description, numerous specific details are set forth, such as specific polishing pad designs and compositions, in order to provide a thorough understanding of embodiments of the present invention. It will be apparent to one skilled in the art that embodiments of the present invention may be practiced without these specific details. In other instances, well-known processing techniques, such as details concerning the combination of a slurry with a polishing pad to perform chemical mechanical planarization (CMP) of a semiconductor substrate, are not described in detail in order to not unnecessarily obscure embodiments of the present invention. Furthermore, it is to be understood that the various embodiments shown in the figures are illustrative representations and are not necessarily drawn to scale.

One or more embodiments described herein are directed to the fabrication of polishing pads having a low density of less than approximately 0.6 grams/cubic centimeter (g/cc) and, more particularly, a low density of less than approximately 0.5 g/cc. The resulting pads are based on a polyurethane material having a closed cell porosity which provides for the low density. The low density pads may be used, e.g., as buff polishing pads or as polishing pads designed for special chemical mechanical polishing (CMP) applications such as liner/barrier removal. Polishing pads described herein may, in some embodiments, be fabricated to have a density as low as in the range of 0.3 g/cc to 0.5 g/cc, such as approximately 0.357 g/cc. In a particular embodiment, a low density pad has a density as low as approximately 0.2 g/cc.

To provide context, a typical CMP pad has a density around 0.7 to 0.8 g/cc, and is generally at least higher than 0.5 g/cc. Conventionally, a typical CMP buff pad has a "poromeric" design using large cells open to the surface. A composite polyurethane skin is included on a support, such as in the case of a POLITEX polishing pad. Conventionally, buff pad are very soft and low density made with open cell porosity (e.g., a fiber pad and "poromeric" pad). Such pads typically are associated with two fundamental issues for CMP: short life time and less consistent performance as compared with conventional closed cell polyurethane (but higher density) CMP pads. Figures 1A and 1B are a top down view and cross-sectional view, respectively, of a POLITEX polishing pad, in accordance with the prior art. Referring to Figure 1A, a portion 100A of a POLITEX polishing pad is shown as magnified 300 times in a scanning electron microscope (SEM) image. Referring to Figure 1B, a portion 100B of a POLITEX polishing pad is shown as magnified 100 times in a scanning electron microscope (SEM) image. Referring to both Figures 1A and 1B, the open pore structure of the prior art pad is readily visible.

WO 2013/ 058183 A1 discloses a method of fabricating a polishing pad, the method comprising mixing a pre-polymer and a chain extender or cross-linker with a plurality of microelements to form a mixture, each of the plurality of microelements having an initial size, and heating, in a formation mold, the mixture to provide a molded polishing body comprising a thermoset polyurethane material and a plurality of closed cell pores dispersed in the thermoset polyurethane material, the plurality of closed cell pores formed by expanding each of the plurality of microelements to a final, larger, size during the heating.

US 5 885 312 discloses the application of unexpanded and pre-expanded microelements in combination in a mixture with epoxy-novolac resin.

More generally, one of the fundamental challenges is to fabricate a closed cell polyurethane pad having high porosity and low density. Our own investigations in the fabrication of low density polyurethane pads by a molding or casting process has shown difficulty in merely adding increased volumes of a porogen into a pad formulation mixture to ultimately provide closed cell pores in the pad material based on the added porogen. In particular, adding more porogen than for a typical pad formulation can increase the viscosity of the formulation to levels unmanageable for a casting or molding process. The case can be particularly difficult for the inclusion of pre-expanded porogens or porogens that retain essentially the same volume throughout the molding or casting process. In accordance with an embodiment of the present invention, un-expanded porogens or porogens that increase volume throughout the molding or casting process are included in a pad formulation for ultimate for generation. In one such embodiment, however, if all final closed cell pores are generated from unexpanded porogens, the viscosity of the formulation may be too low for manageability in casting or molding. As such, according to the invention, in addition forming a formulation to include un-expanded porogens or porogens that increase volume throughout the molding or casting process, pre-expanded porogens are also included to enable viscosity tuning of the pad formulation.

Accordingly, in an embodiment not according to the invention, Unexpanded Porogen Filler or Underexpanded Porogen Filler (both referred to as UPF) that expands at above ambient temperature is used to create porosity in a polishing pad during manufacture by casting or molding. In one such embodiment, a large quantity of UPF is included in a polyurethane-forming mixture. The UPF expands during the pad casting process and creates a low density pad with closed cell pores. The above approach to creating a polishing pad can have advantages over other techniques that have been used to form low density pads with open cells. For example, fabrication of final pad porosity based solely on gas injection or entrainment may require specialized equipment, and may be accompanied by difficulty in controlling final pad density and difficulty in controlling final pore size and distribution. In another example not according to the invention, fabrication of final pad porosity based solely on in situ gas generation, e.g., water reaction with an isocyanate moiety (NCO) to create CO₂ bubbles can be accompanied by a difficulty in controlling pore size distribution.

According to the present invention, low density polishing pads are fabricated in a molding process. For example, Figures 2A-2G illustrate cross-sectional views of operations used in the fabrication of a polishing pad, in accordance with an embodiment of the present invention.

Referring to Figure 2A, a formation mold 200 is provided. Referring to Figure 2B, a pre-polymer 202 and a curative 204 (a chain extender or cross-linker) are mixed with a plurality of microelements to form a mixture. In an embodiment, the plurality of microelements is a plurality of porogens 206, such as filled or hollow microspheres. In another embodiment, the plurality of microelements is a plurality of gas bubbles or liquid droplets, or both, 208. In another embodiment, the plurality of microelements is a combination of a plurality of porogens 206 and a plurality of gas bubbles or liquid droplets, or both, 208.

Referring to Figure 2C, the resulting mixture 210 from Figure 2B is shown at the base of the formation mold 200. The mixture 210 includes a first plurality of microelements 212, each of the first plurality of microelements having an initial size. A second plurality of microelements 214 are also included in the mixture 210, as described in greater detail below.

Referring to Figure 2D, a lid 216 of the formation mold 200 is brought together with the base of the formation mold 200 and the mixture 210 takes the shape of the formation mold 200. In an embodiment, the mold 200 is degassed upon or during bringing together of the lid 216 and base of the formation mold 200 such that no cavities or voids form within the formation mold 210. It is to be understood that embodiments described herein that describe lowering the lid of a formation mold need only achieve a bringing together of the lid and a base of the formation mold. That is, in some embodiments, a base of a formation mold is raised toward a lid of a formation mold, while in other embodiments a lid of a formation mold is lowered toward a base of the formation mold at the same time as the base is raised toward the lid.

Referring to Figure 2E, the mixture 210 is heated in the formation mold 200. Each of the plurality of microelements 212 is expanded to a final, larger, size 218 during the heating. Additionally, referring to Figure 2F, the heating is used to cure the mixture 210 to provide a partially or fully cured pad material 220 surrounding the microelements 218 and the microelements 214. The curing forms a cross-linked matrix based on the materials of the pre-polymer and the curative.

Referring collectively to Figures 2E and2F, it is to be understood that the ordering of expanding microelements 212 to the final, larger, size 218 and the curing the mixture 210 need not necessarily occur in the order illustrated. In another embodiment, during the heating, the curing of the mixture 210 occurs prior to expanding the microelements 212 to the final, larger, size 218. In another embodiment, during the heating, the curing of the mixture 210 occurs at the same time as expanding the microelements 212 to the final, larger, size 218. In yet another embodiment, two separate heating operations are performed to cure the mixture 210 and to expand the microelements 212 to the final, larger, size 218, respectively.

Referring to Figure 2G, in an embodiment, the above described process is used to provide a low density polishing pad 220. The low density polishing pad 222 is composed of the cured material 220 and includes the expanded microelements 218 and additional microelements 214. The low density polishing pad 222 is composed of a thermoset polyurethane material and the expanded microelements 218 provide a plurality of closed cell pores dispersed in the thermoset polyurethane material. Referring again to Figure 2G, the bottom portion of the Figure is the plan view of the upper cross-sectional view which is taken along the a-a' axis. As seen in the plan view, in an embodiment, the low density polishing pad 222 has a polishing surface 228 having a groove pattern therein. In one particular embodiment, as shown, the groove pattern includes radial grooves 226 and concentric circular grooves 228.

Referring again to Figures 2D and 2E, in an embodiment, each of the plurality of microelements 212 is expanded to the final size 218 by increasing a volume of each of the plurality of microelements by a factor approximately in the range of 3 - 1000. In an embodiment, each of the plurality of microelements 212 is expanded to the final size 214 to provide a final diameter of each of the plurality of microelements 218 approximately in the range of 10-200 microns. In an embodiment, each of the plurality of microelements 212 is expanded to the final size 218 by reducing a density of each of the plurality of microelements 212 by a factor approximately in the range of 3-1000. In an embodiment, each of the plurality of microelements 212 is expanded to the final size 218 by forming an essentially spherical shape for each of the plurality of microelements 218 of the final size.

In an embodiment, the plurality of microelements 212 is an added porogen, gas bubble or liquid bubble that is then expanded within the pad material formulation to form closed cell pores within a finished polishing pad material. In one such embodiment, the plurality of closed cell pores is a plurality of larger porogens formed by expanding corresponding smaller porogens. For example, the term "porogen" may be used to indicate micro- or nano-scale spherical or somewhat spherical particles with "hollow" centers. The hollow centers are not filled with solid material, but may rather include a gaseous or liquid core. In one embodiment, the plurality of closed cell pores begins as un-expanded gas-filled or liquid-filled EXPANCEL™ distributed throughout a mixture. Upon and/or during forming a polishing pad from the mixture, e.g., by a molding process, the un-expanded gas-filled or liquid-filled EXPANCEL™ becomes expanded. In a specific embodiment, the EXPANCEL™ is filled with pentane. In an embodiment, each of the plurality of closed cell pores has a diameter approximately in the range of 10 - 100 microns in its expanded state, e.g., in the final product. Thus, in an embodiment, each of the plurality of microelements having the initial size includes a physical shell, and each of the plurality of microelements having the final size includes an expanded physical shell. In another embodiment, each of the plurality of microelements 212 having the initial size is a liquid droplet, and each of the plurality of microelements 218 having the final size is a gas bubble. In yet another embodiment, for form the plurality of microelements 218 having the final size, mixing to form the mixture 210 further involves injecting a gas into the pre-polymer and the chain extender or cross-linker, or into a product formed there from. In a specific such embodiment, the pre-polymer is an isocyanate and the mixing further involves adding water to the pre-polymer. The plurality of closed cell pores are discrete from one another. This is in contrast to open cell pores which may be connected to one another through tunnels, such as the case for the pores in a common sponge.

Referring again to Figures 2C-2E, in an embodiment, mixing the pre-polymer 202 and the chain extender or cross-linker 204 with the plurality of microelements 212 further involves mixing with a second plurality of microelements 214 to form the mixture 210. Each of the second plurality of microelements 214 has a size. The heating described in association with Figure 2E is performed at a temperature sufficiently low such that the size of each of the second plurality of microelements 214 is essentially the same before and after the heating, as is depicted in Figure 2E. In a specific such embodiment, the heating is performed at a temperature of approximately 100 degrees Celsius or less, and the second plurality of microelements 214 has an expansion threshold of greater than approximately 130 degrees Celsius. In one other embodiment, the second plurality of microelements 214 has an expansion threshold greater than an expansion threshold of the plurality of microelements 212. In one specific such embodiment, the expansion threshold of the second plurality of microelements 214 is greater than approximately 120 degrees Celsius, and the expansion threshold of the plurality of microelements 212 is less than approximately 110 degrees Celsius. According to the invention during the heating, the microelements 212 expand during to heating to provide expanded microelements 218, while the microelements 214 essentially remain unchanged.

In an embodiment, each of the second plurality of microelements 214 is composed of pre-expanded and gas-filled EXPANCEL™ distributed throughout (e.g., as an additional component in) the polishing pad. That is, any significant expansion that could occur for the microelements 214 is carried out prior to their inclusion in a polishing pad formation, e.g., before being included in mixture 210. In a specific embodiment, the pre-expanded EXPANCEL™ is filled with pentane. In an embodiment, the microelements 214 provide a plurality of closed cell pores (shown again as 214 with little to no change during the molding process) has a diameter approximately in the range of 10 - 100 microns. The resulting plurality of closed cell pores includes pores that are discrete from one another. This is in contrast to open cell pores which may be connected to one another through tunnels, such as the case for the pores in a common sponge.

As described above, increasing porosity by adding more porogen than for a typical pad formulation can increase the viscosity of the formulation to levels unmanageable for a casting or molding process. The case can be particularly difficult for the inclusion of pre-expanded porogens or porogens that retain essentially the same volume throughout the molding or casting process. On the other hand, if all final closed cell pores are generated from unexpanded porogens, the viscosity of the formulation may be too low for manageability in casting or molding. In order to address such situations, in accordance with an embodiment of the present invention, conceptually, a mixture of the pre-polymer 202, the chain extender or cross-linker 204, and the second plurality of microelements 214 has a viscosity. Meanwhile, the mixture of the pre-polymer 202, the chain extender or cross-linker 204, the plurality of microelements 212 having the initial size, and the second plurality of microelements 214 essentially has the same viscosity. That is, the inclusion of the plurality of microelements 212 having the initial (smaller) size has little to no impact on the viscosity of the mixture. In an embodiment, then, a described viscosity for optimal molding conditions may be selected based on the inclusion of the second plurality of microelements with a size that remains essentially constant throughout the molding process. In one such embodiment, then, the viscosity is a predetermined viscosity, and a relative amount of the second plurality of microelements 214 in the mixture 210 is selected based on the predetermined viscosity. And, in one embodiment, the plurality of microelements 212 has little to no effect on the viscosity of the mixture 210.

Referring again to Figure 2E, in an embodiment according to the invention, where two different pluralities of microelements are included, each of the plurality of microelements 218 having the expanded final size is of approximately the same shape and size as each of the plurality of microelements 214 which do not expand through the heating process, as is depicted. It is to be understood, however, that each of the plurality of microelements 218 having the expanded final size need not have the same shape and/or size as each of the plurality of microelements 214. In an embodiment, as described in greater detail below in association with Figures 6A-6C, the resulting molded polishing body of pad 222 includes, as closed cell pores, the plurality of expanded microelements 218 having a first diameter mode with a first peak of size distribution. Also included, also as closed cell pores, is the second plurality of microelements 214 having a second diameter mode with a second, different, peak of size distribution. In one such embodiment, the plurality of closed cell pores of microelements 218 and the second plurality of closed cell pores of microelements 214 provides a total pore volume in the thermoset polyurethane material approximately in the range of 55 - 80 % of the total volume of the thermoset polyurethane material of low density polishing pad 222.

Referring again to Figures 2D-2G in an embodiment, heating the mixture 210 to provide the molded polishing body 222 involves forming the polishing body 222 having a density of less than 0.5 g/cc. In one such embodiment, however, the mixture 210 has a density of greater than 0.5 g/cc prior to the heating. In an embodiment, the pre-polymer 202 is an isocyanate and the chain extender or cross-linker 204 is an aromatic diamine compound, and the polishing pad 222 is composed of a thermoset polyurethane material 220. In one such embodiment, forming mixture 210 further involves adding an opacifying filler to the pre-polymer 202 and the chain extender or cross-linker 204 to ultimately provide an opaque molded polishing body 222. In a specific such embodiment, the opacifying filler is a material such as, but not limited to, boron nitride, cerium fluoride, graphite, graphite fluoride, molybdenum sulfide, niobium sulfide, talc, tantalum sulfide, tungsten disulfide, or Teflon. In an embodiment, as mentioned briefly above, the mixture 210 is only partially cured in the mold 200 and, in one embodiment, is further cured in an oven subsequent to removal from the formation mold 220.

In an embodiment, the polishing pad precursor mixture 210 is used to ultimately form a molded homogeneous polishing body 222 composed of a thermoset, closed cell polyurethane material. In one such embodiment, the polishing pad precursor mixture 210 is used to ultimately form a hard pad and only a single type of curative 204 is used. In another embodiment, the polishing pad precursor mixture 210 is used to ultimately form a soft pad and a combination of a primary and a secondary curative (together providing 210) is used. For example, in a specific embodiment, the pre-polymer 202 includes a polyurethane precursor, the primary curative includes an aromatic diamine compound, and the secondary curative includes an ether linkage. In a particular embodiment, the polyurethane precursor is an isocyanate, the primary curative is an aromatic diamine, and the secondary curative is a curative such as, but not limited to, polytetramethylene glycol, amino-functionalized glycol, or amino-functionalized polyoxypropylene. In an embodiment, a pre-polymer 202, a primary curative, and a secondary curative (together 204) have an approximate molar ratio of 106 parts pre-polymer, 85 parts primary curative, and 15 parts secondary curative, i.e., to provide a stoichiometry of approximately 1:0.96 pre-polymer:curative. It is to be understood that variations of the ratio may be used to provide polishing pads with varying hardness values, or based on the specific nature of the pre-polymer and the first and second curatives.

Referring again to Figure 2G, as described above, in an embodiment, heating in the formation mold 200 involves forming a groove pattern in the polishing surface 224 of the molded polishing body 222. The groove pattern as shown includes radial grooves and concentric circular circumferential grooves. It is to be understood that radial grooves or circumferential grooves may be omitted. Furthermore, the concentric circumferential grooves may instead be polygons, such as nested triangles, squares, pentagons, hexagons, etc. Alternatively, the polishing surface may instead be based on protrusions instead of grooves. Furthermore, a low density polishing pad may be fabricated without grooves in the polishing surface. In one such example, a non-patterned lid of a molding apparatus is used instead of a patterned lid. Or, alternatively, the use of a lid during molding may be omitted. In the case of the use of a lid during molding, the mixture 210 may be heated under a pressure approximately in the range of 0,14 - 0,84 kilograms per square centimeter (2 - 12 pounds per square inch).

In an aspect, a low density pad may be fabricated having closed cell pores. For example, in an embodiment, a polishing pad includes a polishing body having a density of less than 0.6 and composed of a thermoset polyurethane material. A plurality of closed cell pores is dispersed in the thermoset polyurethane material. In a particular embodiment, the density is less than 0.5 g/cc. In an embodiment, the plurality of closed cell pores provides a total pore volume in the thermoset polyurethane material approximately in the range of 55 - 80 % of the total volume of the thermoset polyurethane material. In an embodiment, each of the plurality of closed cell pores is essentially spherical. In an embodiment, the polishing body further includes a first, grooved surface; and a second, flat, surface opposite the first surface, as described in association with Figure 2G. In an embodiment, the polishing body is a homogeneous polishing body, as is described in greater detail below.

In one exemplary embodiment, each of the plurality of closed cell pores includes a physical shell composed of a material different from the thermoset polyurethane material. In such a case, the closed cell pores may be fabricated by including a porogen in a mixture that is molded for ultimate pad fabrication, as described above.

In another exemplary embodiment, each of the plurality of closed cell pores includes a physical shell composed of a material different from the thermoset polyurethane material. The physical shells of a first portion of the plurality of closed cell pores are composed of a material different than the physical shells of a second portion of the plurality of closed cell pores. The closed cell pores are fabricated by including two types of porogens (expanded and unexpanded) in a mixture that is molded for ultimate pad fabrication, as described above.

In another exemplary embodiment, each of only a portion of the plurality of closed cell pores includes a physical shell composed of a material different from the thermoset polyurethane material. In such a case, the closed cell pores may be fabricated by including both porogens and gas bubbles or liquid drops in a mixture that is molded for ultimate pad fabrication, as described above.

In another exemplary embodiment, each of the plurality of closed cell pores does not include a physical shell of a material different from the thermoset polyurethane material. In such a case, the closed cell pores may be fabricated by including gas bubbles or liquid drops, or both, in a mixture that is molded for ultimate pad fabrication, as described above.

Figure 3 illustrates cross-sectional views at 100x and 300x magnification of a low density polishing pad 300 including closed cell pores which are all based on a porogen filler, in accordance with an embodiment of the present invention. Referring to Figure 3, all pores shown are formed from a porogen and, as such, all include a physical shell. A portion of the pores is formed from a pre-expanded Expancel porogen. Another portion is formed from an unexpanded Expancel porogen which expanded during a molding process used to fabricate polishing pad 300. The un-expanded Expancel expands at low temperature by design. The molding or casting process temperature is above the expansion temperature and the Expancel rapidly expands during the molding or casting. The density of pad 300 is approximately 0.45 and all pores in the pad are closed cell pores.

Figure 4 illustrates cross-sectional views at 100x and 300x magnification of a low density polishing pad 400 including closed cell pores, a portion of which based on a porogen filler and a portion of which is based on gas bubbles, in accordance with an embodiment of the present invention. Referring to Figure 4, the small pores shown are formed from a porogen and, as such, include a physical shell. More specifically, the small pores are formed from a pre-expanded Expancel porogen. The large pores are formed using a gas. More specifically, the large pores are formed using a small quantity of water and surfactant injected into a pad formulation mixture just prior to molding or casting. During the chemical reaction for chain extension, there is a competing chemical reaction of the water with NCO to form CO₂ and create pores. It is to be understood that the surfactant type and concentration, as well as catalyst type and level, controls pore size and the closes/open cell pore ratio. The density of pad 400 is approximately 0.37 and a significant majority of the pores in the pad are closed cell pores.

In an aspect, a distribution of pore diameters in a polishing pad can have a bell curve or mono-modal distribution. For example, Figure 5A illustrates a plot of population as a function of pore diameter for a broad mono-modal distribution of pore diameters in a low density polishing pad, in accordance with an embodiment of the present invention. Referring to plot 500A of Figure 5A, the mono-modal distribution may be relatively broad. As another example, Figure 5B illustrates a plot of population as a function of pore diameter for a narrow mono-modal distribution of pore diameters in a low density polishing pad, in accordance with an embodiment of the present invention. Referring to plot 500B of Figure 5B, the mono-modal distribution may be relatively narrow. In either the narrow distribution or the broad distribution, only one maximum diameter population, such as a maximum population at 40 microns (as shown as an example), is provided in the polishing pad.

In another aspect, a low density polishing pad may instead be fabricated with a bimodal distribution of pore diameters. As an example, Figure 6A illustrates a cross-sectional view of a low density polishing pad having an approximately 1:1 bimodal distribution of closed-cell pores, in accordance with an embodiment of the present invention.

Referring to Figure 6A, a polishing pad 600 includes a homogeneous polishing body 601. The homogeneous polishing body 601 is composed of a thermoset polyurethane material with a plurality of closed cell pores 602 disposed in the homogeneous polishing body 601. The plurality of closed cell pores 602 has a multi-modal distribution of diameters. In an embodiment, the multi-modal distribution of diameters is a bimodal distribution of diameters including a small diameter mode 604 and a large diameter mode 606, as depicted in Figure 6A.

In an embodiment, the plurality of closed cell pores 602 includes pores that are discrete from one another, as depicted in Figure 6A. This is in contrast to open cell pores which may be connected to one another through tunnels, such as the case for the pores in a common sponge. In one embodiment, each of the closed cell pores includes a physical shell, such as a shell of a porogen. In another embodiment, however, some or all of the closed cell pores does not include a physical shell. In an embodiment, the plurality of closed cell pores 602, and hence the multi-modal distribution of diameters, is distributed essentially evenly and uniformly throughout the thermoset polyurethane material of homogeneous polishing body 601, as depicted in Figure 6A.

In an embodiment, the bimodal distribution of pore diameters of the plurality of closed cell pores 602 may be approximately 1:1, as depicted in Figure 6A. To better illustrate the concept, Figure 6B illustrates a plot 620 of population as a function of pore diameter for a narrow distribution of pore diameters in the polishing pad of Figure 6A, in accordance with an embodiment of the present invention. Figure 6C illustrates a plot 630 of population as a function of pore diameter for a broad distribution of pore diameters in the polishing pad of Figure 6A, in accordance with an embodiment of the present invention.

Referring to Figures 6A-6C, the diameter value for the maximum population of the large diameter mode 606 is approximately twice the diameter value of the maximum population of the small diameter mode 604. For example, in one embodiment, the diameter value for the maximum population of the large diameter mode 606 is approximately 40 microns and the diameter value of the maximum population of the small diameter mode 604 is approximately 20 microns, as depicted in Figures 6B and 6C. As another example, the diameter value for the maximum population of the large diameter mode 606 is approximately 80 microns and the diameter value of the maximum population of the small diameter mode 604 is approximately 40 microns.

Referring to plot 620 of Figure 6B, in one embodiment, the distributions of pore diameters are narrow. In a specific embodiment, the population of the large diameter mode 606 has essentially no overlap with the population of the small diameter mode 604. However, referring to plot 630 of Figure 6C, in another embodiment, the distributions of pore diameters are broad. In a specific embodiment, the population of the large diameter mode 606 overlaps with the population of the small diameter mode 604. It is to be understood that, a bimodal distribution of pore diameters need not be 1:1, as is described above in association with Figures 6A-6C. Also, a bimodal distribution of pore diameters need not be uniform. In another embodiment, the multi-modal distribution of diameters of closed cell pores is graded throughout the thermoset polyurethane material with a gradient from the first, grooved surface to the second, flat surface. In one such embodiment, the graded multi-modal distribution of diameters is a bimodal distribution of diameters including a small diameter mode proximate to the first, grooved surface, and a large diameter mode proximate to the second, flat surface.

In an embodiment, then, low density polishing pad has a plurality of closed cell pores with a bi-modal distribution of diameters having a first diameter mode with a first peak of size distribution and a second diameter mode with a second, different, peak of size distribution. In one such embodiment, the closed cell pores of the first diameter mode each include a physical shell composed of a material different from the thermoset polyurethane material. In a specific such embodiment, the closed cell pores of the second diameter mode each include a physical shell composed a material different from the thermoset polyurethane material. In a particular such embodiment, the physical shell of each of the closed cell pores of the second diameter mode is composed of a material different from the material of the physical shells of the closed cell pores of the first diameter mode.

In an embodiment, the first peak of size distribution of the first diameter mode has a diameter approximately in the range of 10 - 50 microns, and the second peak of size distribution of the second diameter mode has a diameter approximately in the range of 10 - 150 microns. In an embodiment, the first diameter mode overlaps with the second diameter mode. In another embodiment, however, the first diameter mode has essentially no overlap with the second diameter mode. In an embodiment, a total population in count number of the first diameter mode is not equal to a total population in count number of the second diameter mode. In another embodiment, however, a total population in count number of the first diameter mode is approximately equal to a total population in count number of the second diameter mode. In an embodiment, the bi-modal distribution of diameters is distributed essentially evenly throughout the thermoset polyurethane material. In another embodiment, however, the bi-modal distribution of diameters is distributed in a graded fashion throughout the thermoset polyurethane material.

In an embodiment, low density polishing pads described herein, such as polishing pad 222, 300 or 400, or the above described variations thereof, are suitable for polishing substrates. In one such embodiment, the polishing pad is used as a buff pad. The substrate may be one used in the semiconductor manufacturing industry, such as a silicon substrate having device or other layers disposed thereon. However, the substrate may be one such as, but not limited to, a substrates for MEMS devices, reticles, or solar modules. Thus, reference to "a polishing pad for polishing a substrate," as used herein, is intended to encompass these and related possibilities.

Low density polishing pads described herein, such as polishing pad 222, 300 or 400, or the above described variations thereof, may be composed of a homogeneous polishing body of a thermoset polyurethane material. In an embodiment, the homogeneous polishing body is composed of a thermoset, closed cell polyurethane material. In an embodiment, the term "homogeneous" is used to indicate that the composition of a thermoset, closed cell polyurethane material is consistent throughout the entire composition of the polishing body. For example, in an embodiment, the term "homogeneous" excludes polishing pads composed of, e.g., impregnated felt or a composition (composite) of multiple layers of differing material. In an embodiment, the term "thermoset" is used to indicate a polymer material that irreversibly cures, e.g., the precursor to the material changes irreversibly into an infusible, insoluble polymer network by curing. For example, in an embodiment, the term "thermoset" excludes polishing pads composed of, e.g., "thermoplast" materials or "thermoplastics" - those materials composed of a polymer that turns to a liquid when heated and returns to a very glassy state when cooled sufficiently. It is noted that polishing pads made from thermoset materials are typically fabricated from lower molecular weight precursors reacting to form a polymer in a chemical reaction, while pads made from thermoplastic materials are typically fabricated by heating a pre-existing polymer to cause a phase change so that a polishing pad is formed in a physical process. Polyurethane thermoset polymers are selected for fabricating polishing pads described herein based on their stable thermal and mechanical properties, resistance to the chemical environment, and tendency for wear resistance.

In an embodiment, the homogeneous polishing body, upon conditioning and/or polishing, has a polishing surface roughness approximately in the range of 1 - 5 microns root mean square. In one embodiment, the homogeneous polishing body, upon conditioning and/or polishing, has a polishing surface roughness of approximately 2.35 microns root mean square. In an embodiment, the homogeneous polishing body has a storage modulus at 25 degrees Celsius approximately in the range of 30 - 120 megaPascals (MPa). In another embodiment, the homogeneous polishing body has a storage modulus at 25 degrees Celsius approximately less than 30 megaPascals (MPa). In one embodiment, the homogeneous polishing body has a compressibility of approximately 2.5%.

The low density polishing pads described herein, such as polishing pad 222, 300 or 400, or the above described variations thereof, include a molded homogeneous polishing body. The term "molded" is used to indicate that a homogeneous polishing body is formed in a formation mold, as described in more detail above in association with Figures 2A-2G.

In an embodiment, the homogeneous polishing body is opaque. In one embodiment, the term "opaque" is used to indicate a material that allows approximately 10% or less visible light to pass. In one embodiment, the homogeneous polishing body is opaque in most part, or due entirely to, the inclusion of an opacifying filler throughout (e.g., as an additional component in) the homogeneous thermoset, closed cell polyurethane material of the homogeneous polishing body. In a specific embodiment, the opacifying filler is a material such as, but not limited to, boron nitride, cerium fluoride, graphite, graphite fluoride, molybdenum sulfide, niobium sulfide, talc, tantalum sulfide, tungsten disulfide, or Teflon.

The sizing of the low density polishing pads, such as pads 222, 300 or 400, may be varied according to application. Nonetheless, certain parameters may be used to fabricate polishing pads compatible with conventional processing equipment or even with conventional chemical mechanical processing operations. For example, in accordance with an embodiment of the present invention, a low density polishing pad has a thickness approximately in the range of 0.075 inches to 0.130 inches, e.g., approximately in the range of 1.9 - 3.3 millimeters. In one embodiment, a low density polishing pad has a diameter approximately in the range of 20 inches to 30.3 inches, e.g., approximately in the range of 50 - 77 centimeters, and possibly approximately in the range of 10 inches to 42 inches, e.g., approximately in the range of 25 - 107 centimeters.

In another embodiment of the present invention, a low density polishing pad described herein further includes a local area transparency (LAT) region disposed in the polishing pad. In an embodiment, the LAT region is disposed in, and covalently bonded with, the polishing pad. Examples of suitable LAT regions are described in U.S. patent application 12/657,135 filed on January 13, 2010, assigned to NexPlanar Corporation, and U.S. patent application 12/895,465 filed on September 30, 2010, assigned to NexPlanar Corporation. In an alternative or additional embodiment, a low density polishing pad further includes an aperture disposed in the polishing surface and polishing body. The aperture can accommodate, e.g., a detection device included in a platen of a polishing tool. An adhesive sheet is disposed on the back surface of the polishing body. The adhesive sheet provides an impermeable seal for the aperture at the back surface of the polishing body. Examples of suitable apertures are described in U.S. patent application 13/184,395 filed on July 15, 2011, assigned to NexPlanar Corporation. In another embodiment, a low density polishing pad further includes a detection region for use with, e.g., an eddy current detection system. Examples of suitable eddy current detection regions are described in U.S. patent application 12/895,465 filed on September 30, 2010, assigned to NexPlanar Corporation.

Low density polishing pads described herein, such as polishing pad 222, 300 or 400, or the above described variations thereof, may further include a foundation layer disposed on the back surface of the polishing body. In one such embodiment, the result is a polishing pad with bulk or foundation material different from the material of the polishing surface. In one embodiment, a composite polishing pad includes a foundation or bulk layer fabricated from a stable, essentially non-compressible, inert material onto which a polishing surface layer is disposed. A harder foundation layer may provide support and strength for pad integrity while a softer polishing surface layer may reduce scratching, enabling decoupling of the material properties of the polishing layer and the remainder of the polishing pad. Examples of suitable foundation layers are described in U.S. patent application 13/306,845 filed on November 29, 2011, assigned to NexPlanar Corporation.

Low density polishing pads described herein, such as polishing pad 222, 300 or 400, or the above described variations thereof, may further include a sub pad disposed on the back surface of the polishing body, e.g., a conventional sub pad as known in the CMP art. In one such embodiment, the sub pad is composed of a material such as, but not limited to, foam, rubber, fiber, felt or a highly porous material.

Referring again to Figure 2G as a foundation for description, individual grooves of a groove pattern formed in a low density polishing pad such as those described herein may be from 0.10 to 2.54 mm (about 4 to about 100 mils) deep at any given point on each groove. In some embodiments, the grooves are 0.25 to 1.27 mm (about 10 to about 50 mils deep) at any given point on each groove. The grooves may be of uniform depth, variable depth, or any combinations thereof. In some embodiments, the grooves are all of uniform depth. For example, the grooves of a groove pattern may all have the same depth. In some embodiments, some of the grooves of a groove pattern may have a certain uniform depth while other grooves of the same pattern may have a different uniform depth. For example, groove depth may increase with increasing distance from the center of the polishing pad. In some embodiments, however, groove depth decreases with increasing distance from the center of the polishing pad. In some embodiments, grooves of uniform depth alternate with grooves of variable depth.

Individual grooves of a groove pattern formed in a low density polishing pad such as those described herein may be from 0.05 to 2.54 mm (about 2 to about 100 mils) wide at any given point on each groove. In some embodiments, the grooves are 0.38 to 1.27 mm (about 15 to about 50 mils) wide at any given point on each groove. The grooves may be of uniform width, variable width, or any combinations thereof. In some embodiments, the grooves of are all of uniform width. In some embodiments, however, some of the grooves of a concentric have a certain uniform width, while other grooves of the same pattern have a different uniform width. In some embodiments, groove width increases with increasing distance from the center of the polishing pad. In some embodiments, groove width decreases with increasing distance from the center of the polishing pad. In some embodiments, grooves of uniform width alternate with grooves of variable width.

In accordance with the previously described depth and width dimensions, individual grooves of the groove patterns described herein, including grooves at or near a location of an aperture in a polishing pad, may be of uniform volume, variable volume, or any combinations thereof. In some embodiments, the grooves are all of uniform volume. In some embodiments, however, groove volume increases with increasing distance from the center of the polishing pad. In some other embodiments, groove volume decreases with increasing distance from the center of the polishing pad. In some embodiments, grooves of uniform volume alternate with grooves of variable volume.

Grooves of the groove patterns described herein may have a pitch 0.76 to 25.4 mm (about 30 to about 1000 mils). In some embodiments, the grooves have a pitch of 3.18 mm (about 125 mils). For a circular polishing pad, groove pitch is measured along the radius of the circular polishing pad. In CMP belts, groove pitch is measured from the center of the CMP belt to an edge of the CMP belt. The grooves may be of uniform pitch, variable pitch, or in any combinations thereof. In some embodiments, the grooves are all of uniform pitch. In some embodiments, however, groove pitch increases with increasing distance from the center of the polishing pad. In some other embodiments, groove pitch decreases with increasing distance from the center of the polishing pad. In some embodiments, the pitch of the grooves in one sector varies with increasing distance from the center of the polishing pad while the pitch of the grooves in an adjacent sector remains uniform. In some embodiments, the pitch of the grooves in one sector increases with increasing distance from the center of the polishing pad while the pitch of the grooves in an adjacent sector increases at a different rate. In some embodiments, the pitch of the grooves in one sector increases with increasing distance from the center of the polishing pad while the pitch of the grooves in an adjacent sector decreases with increasing distance from the center of the polishing pad. In some embodiments, grooves of uniform pitch alternate with grooves of variable pitch. In some embodiments, sectors of grooves of uniform pitch alternate with sectors of grooves of variable pitch.

Polishing pads described herein may be suitable for use with a variety of chemical mechanical polishing apparatuses. As an example, Figure 7 illustrates an isometric side-on view of a polishing apparatus compatible with a low density polishing pad, in accordance with an embodiment of the present invention.

Referring to Figure 7, a polishing apparatus 700 includes a platen 704. The top surface 702 of platen 704 may be used to support a low density polishing pad. Platen 704 may be configured to provide spindle rotation 706 and slider oscillation 708. A sample carrier 710 is used to hold, e.g., a semiconductor wafer 711 in place during polishing of the semiconductor wafer with a polishing pad. Sample carrier 710 is further supported by a suspension mechanism 712. A slurry feed 714 is included for providing slurry to a surface of a polishing pad prior to and during polishing of the semiconductor wafer. A conditioning unit 790 may also be included and, in one embodiment, includes a diamond tip for conditioning a polishing pad.

Thus, low density polishing pads and methods of fabricating low density polishing pads have been disclosed.

## Claims

1. A method of fabricating a polishing pad, the method comprising:
mixing a pre-polymer (202) and a chain extender or cross-linker (204) with a plurality of unexpanded microelements (212) and a plurality of pre-expanded microelements (214) to form a mixture, each of the plurality of unexpanded microelements (212) having an initial size; and
heating the mixture in a formation mold (200) to provide a molded polishing body (220) comprising a thermoset polyurethane material and a first plurality of closed cell pores (218) and a second plurality of closed cell pores (214) dispersed in the thermoset polyurethane material, the first plurality of closed cell pores (218) formed by expanding each of the plurality of unexpanded microelements (212) to a final, larger size during the heating, wherein the heating is performed at a temperature sufficiently low such that a size of each of the plurality of pre-expanded microelements (214) is essentially the same before and after the heating to provide the second plurality of closed cell pores (214) in the molded polishing body.

2. The method of claim 1, wherein expanding each of the plurality of unexpanded microelements to the final size comprises:
increasing a volume of each of the plurality of unexpanded microelements by a factor approximately in the range of 3 - 1000; or
providing a final diameter of each of the plurality of unexpanded microelements approximately in the range of 10-200 microns; or
reducing a density of each of the plurality of unexpanded microelements by a factor approximately in the range of 3-1000; or
forming an essentially spherical shape for each of the plurality of unexpanded microelements of the final size.

3. The method of claim 1, wherein the heating is performed at a temperature of approximately 100 degrees Celsius or less, and wherein the plurality of pre-expanded microelements (214) has an expansion threshold of greater than approximately 130 degrees Celsius.

4. The method of claim 1, wherein the plurality of pre-expanded microelements (214) has an expansion threshold greater than an expansion threshold of the plurality of unexpanded microelements.

5. The method of claim 4, wherein the expansion threshold of the plurality of pre-expanded microelements (214) is greater than approximately 120 degrees Celsius, and the expansion threshold of the plurality of unexpanded microelements (212) is less than approximately 110 degrees Celsius.

6. The method of claim 1, wherein a mixture of the pre-polymer, the chain extender or cross-linker, and the plurality of pre-expanded microelements (214) has a viscosity, and the mixture of the pre-polymer, the chain extender or cross-linker, the plurality of unexpanded microelements (212) having the initial size, and the plurality of pre-expanded microelements (214) essentially has the same viscosity.

7. The method of claim 6, wherein either:
the viscosity is a predetermined viscosity, and a relative amount of the plurality of pre-expanded microelements in the mixture is selected based on the predetermined viscosity; or
the plurality of unexpanded microelements has little to no effect on the viscosity of the mixture.

8. The method of claim 1, wherein heating provides the molded polishing body comprising the thermoset polyurethane material, the first plurality of closed cell pores dispersed in the thermoset polyurethane material and formed by expanding each of the plurality of unexpanded microelements to the final size having a first diameter mode with a first peak of size distribution, and the second plurality of closed cell pores dispersed in the thermoset polyurethane material and formed from the plurality of pre-expanded microelements having a second diameter mode with a second, different, peak of size distribution;
optionally wherein the first plurality of closed cell pores and the second plurality of closed cell pores provides a total pore volume in the thermoset polyurethane material approximately in the range of 55 - 80 % of the total volume of the thermoset polyurethane material.

9. The method of claim 1, wherein heating the mixture to provide the molded polishing body comprises forming the polishing body having a density of less than 0.5 g/cc;
optionally wherein the mixture has a density of greater than 0.5 g/cc prior to the heating

10. The method of claim 1, wherein the mixing further comprises either:
injecting a gas into the pre-polymer and the chain extender or cross-linker, or into a product formed there from; or
adding an opacifying filler to the pre-polymer and the chain extender or cross-linker to provide an opaque molded polishing body.

11. The method of claim 1, wherein the pre-polymer is an isocyanate and the mixing further comprises adding water to the pre-polymer.

12. The method of claim 1, wherein mixing the pre-polymer and the chain extender or cross-linker comprises mixing an isocyanate and an aromatic diamine compound, respectively.

13. The method of claim 1, wherein heating the mixture comprises first partially curing in the formation mold and then further curing in an oven.

14. The method of claim 1, wherein heating in the formation mold comprises forming a groove pattern in a polishing surface of the molded polishing body.

15. The method of claim 1, wherein each of the plurality of unexpanded microelements having the initial size comprises a physical shell, and wherein each of the plurality of microelements having the final size comprises an expanded physical shell.

## Patentansprüche

1. Verfahren des Herstellens eines Polierkissens, wobei das Verfahren Folgendes umfasst:
Mischen eines Prepolymers (202) und eines Kettenverlängerers oder Vernetzungsmittels (204) mit einer Vielzahl von nicht expandierten Mikroelementen (212) und einer Vielzahl von vorexpandierten Mikroelementen (214), um ein Gemisch zu bilden, wobei jedes der Vielzahl von nicht expandierten Mikroelementen (212) eine Anfangsgröße hat; und
Erwärmen des Gemischs in einer Bildungsform (200), um einen geformten Polierkörper (220) bereitzustellen, umfassend ein wärmegehärtetes Polyurethanmaterial und eine erste Vielzahl von geschlossenzelligen Poren (218) und eine zweite Vielzahl von geschlossenzelligen Poren (214), die in dem wärmegehärteten Polyurethanmaterial dispergiert sind, wobei die erste Vielzahl von geschlossenzelligen Poren (218) durch Expandieren von jeder der Vielzahl von nicht expandierten Mikrozellen (212) zu einer finalen, größeren Größe während des Erwärmens gebildet ist, wobei die Erwärmung bei einer Temperatur durchgeführt wird, die ausreichend niedrig ist, sodass eine Größe von jedem der Vielzahl von vorexpandierten Mikroelementen (214) im Wesentlichen vor und nach der Erwärmung gleich ist, um die zweite Vielzahl von geschlossenzelligen Poren (214) in dem geformten Polierkörper bereitzustellen.

2. Verfahren nach Anspruch 1, wobei das Expandieren von jedem der Vielzahl von nicht expandierten Mikroelementen auf die finale Größe Folgendes umfasst:
Erhöhen eines Volumens von jedem der Vielzahl von nicht expandierten Mikroelementen um einen Faktor etwa im Bereich von 3-1000; oder
Bereitstellen eines finalen Durchmessers von jedem der Vielzahl von nicht expandierten Mikroelementen etwa im Bereich von 10-200 Mikron; oder
Verringern einer Dichte von jedem der Vielzahl von nicht expandierten Mikroelementen um einen Faktor etwa im Bereich von 3-1000; oder
Bilden einer im Wesentlichen kugelförmigen Gestalt für jedes der Vielzahl von nicht expandierten Mikroelementen mit der finalen Größe.

3. Verfahren nach Anspruch 1, wobei die Erwärmung bei einer Temperatur von etwa 100 Grad Celsius oder weniger durchgeführt wird und wobei die Vielzahl von vorexpandierten Mikroelementen (214) einen Expansionsschwellenwert von höher als etwa 130 Grad Celsius hat.

4. Verfahren nach Anspruch 1, wobei die Vielzahl von vorexpandierten Mikroelementen (214) einen Expansionsschwellenwert hat, der höher als ein Expansionsschwellenwert der Vielzahl von nicht expandierten Mikroelementen ist.

5. Verfahren nach Anspruch 4, wobei der Expansionsschwellenwert der Vielzahl von vorexpandierten Mikroelementen (214) höher als etwa 120 Grad Celsius ist und der Expansionsschwellenwert der Vielzahl von nicht expandierten Mikroelementen (212) niedriger als etwa 110 Grad Celsius ist.

6. Verfahren nach Anspruch 1, wobei ein Gemisch aus dem Prepolymer, dem Kettenverlängerer oder Vernetzungsmittel und der Vielzahl von vorexpandierten Mikroelementen (214) eine Viskosität hat; und
das Gemisch aus dem Prepolymer, dem Kettenverlängerer oder Vernetzungsmittel, der Vielzahl von nicht expandierten Mikroelementen (212), die die Anfangsgröße haben, und der Vielzahl von vorexpandierten Mikroelementen (214) im Wesentlichen die gleiche Viskosität hat.

7. Verfahren nach Anspruch 6, wobei entweder:
die Viskosität eine vorbestimmte Viskosität ist und eine relative Menge der Vielzahl von vorexpandierten Mikroelementen in dem Gemisch ausgewählt ist basierend auf der vorbestimmten Viskosität; oder
die Vielzahl von nicht expandierten Mikroelementen wenig bis keine Auswirkung auf die Viskosität des Gemischs hat.

8. Verfahren nach Anspruch 1, wobei Erwärmen den geformten Polierkörper bereitstellt, umfassend das wärmegehärtete Polyurethanmaterial, die erste Vielzahl von geschlossenzelligen Poren, die in dem wärmegehärteten Polyurethanmaterial dispergiert und durch Expandieren von jedem der Vielzahl von nicht expandierten Mikroelementen auf die finale Größe mit einem ersten Durchmessermodus mit einer ersten Spitze von Größenverteilung gebildet sind, und die zweite Vielzahl von geschlossenzelligen Poren, die in dem wärmegehärteten Polyurethanmaterial dispergiert und aus der Vielzahl von vorexpandierten Mikroelementen mit einem zweiten Durchmessermodus mit einer zweiten anderen Spitze von Größenverteilung gebildet sind;
optional wobei die erste Vielzahl von geschlossenzelligen Poren und die zweite Vielzahl von geschlossenzelligen Poren ein Porengesamtvolumen in dem wärmegehärteten Polyurethanmaterial etwa im Bereich von 55-80 % des Gesamtvolumens des wärmegehärteten Polyurethanmaterials bereitstellen.

9. Verfahren nach Anspruch 1, wobei das Erwärmen des Gemischs, um den geformten Polierkörper bereitzustellen, das Bilden des Polierkörpers mit einer Dichte von weniger als 0,5 g/cc umfasst;
optional wobei das Gemisch eine Dichte von größer als 0,5 g/cc vor dem Erwärmen hat.

10. Verfahren nach Anspruch 1, wobei das Gemisch ferner eines aus Folgendem umfasst:
Injizieren eines Gases in das Prepolymer und den Kettenverlängerer oder das Vernetzungsmittel oder in ein Produkt, das daraus gebildet ist; oder
Hinzufügen eines trübenden Füllstoffs zu dem Prepolymer und dem Kettenverlängerer oder dem Vernetzungsmittel, um einen opaken geformten Polierkörper bereitzustellen.

11. Verfahren nach Anspruch 1, wobei das Prepolymer ein Isocyanat ist und das Mischen ferner das Hinzufügen von Wasser zu dem Prepolymer umfasst.

12. Verfahren nach Anspruch 1, wobei das Mischen des Prepolymers und des Kettenverlängerers oder Vernetzungsmittels das Mischen eines Isocyanats bzw. einer aromatischen Diaminverbindung umfasst.

13. Verfahren nach Anspruch 1, wobei das Erwärmen des Gemischs zuerst das teilweise Härten in der Bildungsform und dann ferner Härten in einem Ofen umfasst.

14. Verfahren nach Anspruch 1, wobei das Erwärmen in der Bildungsform das Bilden eines Rillenmusters in einer Polierfläche des geformten Polierkörpers umfasst.

15. Verfahren nach Anspruch 1, wobei jedes der Vielzahl von nicht expandierten Mikroelementen mit der Anfangsgröße eine physische Hülle hat und wobei jedes der Vielzahl von Mikroelementen mit der finalen Größe eine expandierte physische Hülle umfasst.

## Revendications

1. Procédé de fabrication d'un tampon de polissage, le procédé comprenant :
le mélange d'un pré-polymère (202) et un prolongateur de chaîne ou un agent de réticulation (204) avec une pluralité de micro-éléments non expansés (212) et une pluralité de micro-éléments pré-expansés (214) pour former un mélange, chacun de la pluralité de micro-éléments non expansés (212) ayant une taille initiale ; et
le chauffage du mélange dans un moule de formation (200) pour obtenir un corps de polissage moulé (220) comprenant un matériau polyuréthane thermodurci et une première pluralité de pores à cellules fermées (218) et une seconde pluralité de pores à cellules fermées (214) dispersés dans le matériau polyuréthane thermodurci, la première pluralité de pores à cellules fermées (218) formés en dilatant chacun de la pluralité de micro-éléments non expansés (212) jusqu'à une taille finale plus grande pendant le chauffage, dans lequel le chauffage étant effectué à une température suffisamment basse pour qu'une taille de chacun de la pluralité de micro-éléments pré-expansés (214) est essentiellement le même avant et après le chauffage pour fournir la seconde pluralité de pores à cellules fermées (214) dans le corps de polissage moulé.

2. Procédé selon la revendication 1, dans lequel l'expansion de chacun de la pluralité de micro-éléments non expansés à la taille finale comprend :
l'augmentation d'un volume de chacun de la pluralité de micro-éléments non expansés d'un facteur approximativement compris entre 3 et 1000 ; ou
la fourniture d'un diamètre final de chacun de la pluralité de micro-éléments non expansés approximativement dans la plage comprise entre 10 et 200 microns ; ou
la réduction d'une densité de chacun de la pluralité de micro-éléments non expansés d'un facteur approximativement compris entre 3 et 1000 ; ou
la formation d'une forme essentiellement sphérique pour chacun de la pluralité de micro-éléments non expansés de la taille finale.

3. Procédé selon la revendication 1, dans lequel le chauffage est effectué à une température d'approximativement 100 degrés Celsius ou moins, et dans lequel la pluralité de micro-éléments pré-expansés (214) a un seuil de dilatation supérieur à environ 130 degrés Celsius.

4. Procédé selon la revendication 1, dans lequel la pluralité de micro-éléments pré-expansés (214) a un seuil de dilatation supérieur à un seuil de dilatation de la pluralité de micro-éléments non expansés.

5. Procédé selon la revendication 4, dans lequel le seuil de dilatation de la pluralité de micro-éléments pré-expansés (214) est supérieur à environ 120 degrés Celsius et le seuil de dilatation de la pluralité de micro-éléments non expansés (212) est inférieur à environ 110 degrés Celsius.

6. Procédé selon la revendication 1, dans lequel un mélange du pré-polymère, de l'allongeur de chaîne ou du réticulant et de la pluralité de micro-éléments pré-expansés (214) a une viscosité, et
le mélange du pré-polymère, de l'allongeur de chaîne ou du réticulant, de la pluralité de micro-éléments non expansés (212) ayant la taille initiale et de la pluralité de micro-éléments pré-expansés (214) a essentiellement la même viscosité.

7. Procédé selon la revendication 6, dans lequel soit :
la viscosité est une viscosité prédéterminée, et une quantité relative de la pluralité de micro-éléments pré-expansés dans le mélange est sélectionnée sur la base de la viscosité prédéterminée ; ou
la pluralité de micro-éléments non expansés n'a que peu ou pas d'effet sur la viscosité du mélange.

8. Procédé selon la revendication 1, dans lequel le chauffage fournit le corps de polissage moulé comprenant le matériau polyuréthane thermodurci, la première pluralité de pores à cellules fermées dispersés dans le matériau polyuréthane thermodurci et formés en dilatant chacun de la pluralité de micro-éléments non expansés à la taille finale ayant un premier mode de diamètre avec un premier pic de distribution de taille, et la seconde pluralité de pores à cellules fermées dispersés dans le matériau de polyuréthane thermodurci et formés à partir de la pluralité de micro-éléments pré-expansés ayant un second mode de diamètre avec un second pic de distribution de taille différent ;
éventuellement, dans lequel la première pluralité de pores à cellules fermées et la seconde pluralité de pores à cellules fermées fournissent un volume de pores total dans le matériau polyuréthane thermodurci approximativement dans la plage de 55 à 80% du volume total du matériau polyuréthane thermodurci.

9. Procédé selon la revendication 1, dans lequel le chauffage du mélange pour fournir le corps de polissage moulé comprend la formation du corps de polissage ayant une densité inférieure à 0,5 g / cc ;
éventuellement dans lequel le mélange a une masse volumique supérieure à 0,5 g / cc avant le chauffage.

10. Procédé selon la revendication 1, dans lequel le mélange comprend en outre soit :
l'injection d'un gaz dans le pré-polymère et l'allongeur de chaîne ou l'agent de réticulation, ou dans un produit formé à partir de ceux-ci ; ou
l'ajout d'une charge opacifiante au pré-polymère et à l'allongeur de chaîne ou à l'agent de réticulation pour obtenir un corps de polissage moulé opaque.

11. Procédé selon la revendication 1, dans lequel le pré-polymère est un isocyanate et le mélange comprend en outre l'addition d'eau au pré-polymère.

12. Procédé selon la revendication 1, dans lequel le mélange du pré-polymère et de l'agent d'extension ou de réticulation de chaîne comprend le mélange d'un isocyanate et d'un composé diamine aromatique, respectivement.

13. Procédé selon la revendication 1, dans lequel le chauffage du mélange comprend d'abord un durcissement partiel dans le moule de formation, puis un durcissement supplémentaire dans un four.

14. Procédé selon la revendication 1, dans lequel le chauffage dans le moule de formation comprend la formation d'un motif de rainure dans une surface de polissage du corps de polissage moulé.

15. Procédé selon la revendication 1, dans lequel chacun de la pluralité de micro-éléments non expansés ayant la taille initiale comprend une coque physique, et dans lequel chacun de la pluralité de micro-éléments ayant la taille finale comprend une coque physique expansée.
